

[54] PROCESS FOR ELECTROLESS  
DEPOSITION OF METALS ON ZIRCONIUM  
MATERIALS

|           |         |                  |            |
|-----------|---------|------------------|------------|
| 3,264,219 | 10/1966 | McGrew .....     | 252/79.3 X |
| 3,667,991 | 6/1972  | Miller .....     | 427/438 X  |
| 3,725,217 | 4/1973  | Hartshorn .....  | 148/6.14 R |
| 4,017,368 | 4/1977  | Wax et al. ..... | 156/656    |

[75] Inventor: Robert E. Donaghy, Wilmington, N.C.

Primary Examiner—Ralph S. Kendall

Attorney, Agent, or Firm—Ivor J. James, Jr.; Sam E. Laub; Samuel E. Turner

[73] Assignee: General Electric Company, San Jose, Calif.

[21] Appl. No.: 729,860

## [57] ABSTRACT

[22] Filed: Oct. 4, 1976

A process for the electroless deposition of a metal layer on an article comprised of zirconium or a zirconium alloy is disclosed. The article is activated in an aged aqueous solution comprising from about 10 to about 20 grams per liter ammonium bifluoride and from about 0.75 to about 2 grams per liter of sulfuric acid. The solution is aged by immersion of pickled zirconium in the solution for at least about 10 minutes. The loosely adhering film formed on the article in the activating step is removed and the article is contacted with an electroless plating solution containing the metal to be deposited on the article upon sufficient contact with the article.

[51] Int. Cl.<sup>2</sup> ..... C23C 3/02[52] U.S. Cl. ..... 427/304; 427/305;  
427/309; 427/437; 427/438; 156/664; 252/79.3;  
176/82; 148/6.24; 148/6.14 R[58] Field of Search ..... 427/304, 305, 437, 438,  
427/309, 6; 148/6.24, 6.14 R; 252/79.3; 176/82;  
156/656, 664

## [56] References Cited

## U.S. PATENT DOCUMENTS

|           |         |                     |            |
|-----------|---------|---------------------|------------|
| 2,928,757 | 3/1960  | Lee et al. ....     | 427/438 X  |
| 2,955,061 | 10/1960 | Jenkins et al. .... | 148/6.14 R |
| 3,029,158 | 4/1962  | Lee ....            | 427/305    |

19 Claims, 1 Drawing Figure





**PROCESS FOR ELECTROLESS DEPOSITION OF METALS ON ZIRCONIUM MATERIALS**

**BACKGROUND OF THE INVENTION**

This invention relates to a process for electroless deposition of a metal layer on zirconium or a zirconium alloy, and more particularly to an improved process for electroless deposition of a metal film such as a copper film on the internal surface of a long hollow cylindrical tube of zirconium or a zirconium alloy.

Nuclear reactors are presently being designed, constructed and operated with the nuclear fuel being contained in fuel elements which can have various geometric shapes, such as plates, tubes, or rods. The fuel material is usually enclosed in a corrosion-resistant, non-reactive, heat conductive container or cladding. The elements are assembled together in a lattice at fixed distances from each other in a coolant flow channel or region forming a fuel assembly, and sufficient fuel assemblies are combined to form the nuclear fission chain reacting assembly or reactor core capable of a self-sustained fission reaction. The core in turn is enclosed within a reactor vessel through which a coolant is passed.

The cladding serves several purposes and two primary purposes are: first, to prevent contact and chemical reactions between the nuclear fuel and the coolant or the moderator if a moderator is present, or both if both coolant and moderator are present; and second, to prevent the radioactive fission products, some of which are gases, from being released from the fuel into the coolant or the moderator or both if both coolant and moderator are present. Common cladding materials are zirconium and its alloys as well as others that are commonly used. The failure of the cladding, i.e., a loss of the leak tightness, can contaminate the coolant or moderator and the associated systems with radioactive long-lived products to a degree which interferes with plant operation.

Problems have been encountered in the operation of nuclear fuel elements which employ certain metals and alloys as the clad material due to mechanical or chemical reactions of these cladding materials under certain circumstances. Zirconium and its alloys, under normal circumstances, are excellent nuclear fuel claddings since they have low neutron absorption cross sections and at temperatures below about 750° F (about 398° C) are strong, ductile, extremely stable and non-reactive in the presence of demineralized water or steam which are commonly used as reactor coolants and moderators.

However, fuel element performance has revealed a problem with the brittle splitting of the cladding due to the combined interactions between the nuclear fuel, the cladding and the fission products produced during nuclear fission reactions. It has been discovered that this brittle splitting is due to localized mechanical stresses resulting from the differential expansion of the fuel into contact with the cladding (i.e., stresses in the cladding are localized at cracks in the nuclear fuel). Corrosive fission products are released from the nuclear fuel and are present at the intersection of the fuel cracks with the cladding surface. Fission products are created in the nuclear fuel during the fission chain reaction occurring during operation of a nuclear reactor. The localized stress is exaggerated by high friction between the fuel and the cladding.

A composite cladding container disclosed in U.S. patent application Ser. No. 522,769, now abandoned, has improved performance and resistance to mechanical and chemical reactions. This application was filed in the names of Gerald M. Gordon and Robert L. Cowan on Nov. 11, 1974 and is assigned to the same assignee as the present invention. The composite cladding container is comprised of an outer layer consisting of zirconium or a zirconium alloy that has bonded on the inside surface of the outer layer a protective layer of a material selected from the group consisting of copper, nickel, iron or alloys thereof. Various methods are disclosed for coating the inside surface of the outer layer of zirconium or a zirconium alloy with the protective layer, and one of the methods involves electroplating. Copper is a particularly preferred material for use as the protective layer.

A novel aqueous electrolytic activating solution and 20 a method for electroplating a metal layer on zirconium and zirconium alloys are disclosed in U.S. Pat. No. 4,017,368. This application was filed in the names of Daniel E. Wax and Robert L. Cowan on Nov. 11, 1974 and is assigned to the same assignee as the present invention. The electroplating method of this invention is particularly suitable for coating the inside surface of zirconium or a zirconium alloy with the protective layer of copper, nickel or iron (as called for in application Ser. No. 522,769, now abandoned). The first step of 30 the process comprises activating the zirconium or zirconium alloy in an aged aqueous electrolytic activating solution comprising from about 10 to about 20 grams per liter of ammonium bifluoride and from 0.75 to about 2 grams per liter of sulfuric acid. The solution is aged by immersion of pickled zirconium in the solution for at 35 least about 10 minutes. The second step of the process comprises electroplating the zirconium material in a plating bath of the metal to be plated on the zirconium material in the presence of an electrode.

Zirconium materials activated in an ammonium bifluoride-sulfuric acid solution have on the surface a first black layer that is highly adherent to the zirconium substrate and is electrically conductive. This first layer is believed to make it possible to initiate electroplating of the zirconium material. These activated zirconium materials also have a second layer on the first layer that is a loosely adhering layer of similar color to the first layer. The presence of this second layer is believed to have an adverse effect on adhesion and to give rise to the possibility of blistering of the coating.

An electroplating process requires the use of an electrode approximately the same length as the piece being plated. The nuclear fuel cladding is a tube of about 14 feet in length and about 0.5 inch in internal diameter. This means that an electrode of about 14 feet in length with about 0.125 inch in diameter is required for an electroplating process. The use of such an electrode can pose problems of shorting.

Further the insertion and withdrawal of an electrode into the cavity of hollow cylindrical tubing during an electrolytic deposition process requires time and can develop problems when attempts are made to automate the process.

Therefore it is desirable to develop an electroless process for depositing a metal layer on the internal surface of zirconium or a zirconium alloy cladding.

## SUMMARY OF THE INVENTION

It has now been discovered that an article comprised of zirconium or a zirconium alloy can be plated with a metal layer of a metal selected from the group consisting of copper and nickel by using an electroless plating process. The first step of the process is activating the article in an aged aqueous activating solution comprised of from about 10 to about 20 grams per liter of ammonium bifluoride and from about 0.75 to about 2 grams per liter of sulfuric acid. The next step of the process is removing the loosely adhering film formed on the article in the activating step. The last step of the process is contacting the article with an electroless plating solution containing the metal to be deposited on the article upon sufficient contact with the article.

The removal of the loosely adhering film formed on the article in the activation step can be done by chemical treatment, ultrasonic treatment or by swabbing the surface with cotton or an organic material. The chemical removal of the film is accomplished by using (a) an aqueous solution comprising from about 2 to about 10 percent fluoboric acid and the balance water, or (b) an aqueous solution comprising from about 2 to about 10 percent hydrofluosilicic acid and the balance water. The ultrasonic removal of the film is accomplished by immersing the article in water and applying ultrasonic energy to the article.

## OBJECTS OF THE INVENTION

It is an object of this invention to provide a process for the electroless plating of an article comprised of zirconium or a zirconium alloy, especially when the article is in the form of a nuclear fuel element cladding comprising a long hollow cylindrical tube of small diameter.

Another object of this invention is to provide a step for removing the loosely adhering film on an article comprised of zirconium or a zirconium alloy after being contacted in an activating solution and prior to being subjected to electroless plating.

Other objects and advantages of this invention will become apparent to the person skilled in the art from the following description of the invention and from the appended claims.

## DESCRIPTION OF THE INVENTION

This invention comprises a process for the electroless deposition of a metal film on an article being comprised of zirconium or a zirconium alloy. The process broadly comprises a step of activating the article, a step of removing any loosely adhering film or films formed on the article in the activation step and a step of contacting the article with an electroless plating solution containing the metal to be deposited on the article upon sufficient contact with the article. The process can also include the optional steps of rinsing the article in water (preferably deionized water) after the activation step, the film removal step and the electroless plating step. The rinsing prevents carry-over on the surface of the article of the solution with which it was in contact so there is no formation of deposits or films on the article from this solution. When the article is to be contacted with another solution, the rinsing also prevents introduction of impurities in that other solution.

A detailed discussion of the process of this invention will now be presented as shown in the FIGURE.

In the first step the article of zirconium or a zirconium alloy is contacted with an aged aqueous activating solution comprising from about 10 to about 20 grams per liter of ammonium bifluoride (preferably a starting amount of about 15 grams per liter ammonium bifluoride) and from about 0.75 to about 2.0 grams per liter of sulfuric acid (preferably a starting amount of about 1.0 grams per liter). The solution is aged by immersion of a piece of pickled zirconium for at least about 10 minutes at ambient temperature. It has been found that solutions outside the foregoing ranges for the ammonium bifluoride component and the sulfuric acid component do not produce good adherent platings on the article.

The article is contacted with the aqueous activating solution for about 1 minute at ambient temperature (approximately 20°-30° C), and the activating solution is stirred or otherwise agitated prior to contacting the article with the solution. The article is ready for immediate use in the following steps of this process or can be stored for several days or longer before being used in the following steps of this process.

An optional step of rinsing the article in water can be practiced, preferably using deionized water, to free the article of any residual traces of the activating solution.

The next step is removing any loosely adhering film (i.e. "smut") formed on the article in the activating step. This step is performed by either (1) contacting the article in a chemical solution so the solution removes the film from the article, (2) using ultrasonic energy to remove the film, or (3) swabbing the surface of the article with a cotton swab or an organic swab such as nylon or polyester. The organic swab can be wrapped around a rubber plug and forced through the article when the article is a hollow tube and the wrapped plug is approximately the same size as the internal diameter of the tube. This leaves the article with a dark adherent electrically conducting surface film or layer of zirconium oxide that can be plated with any of the known electroless metal plating solutions.

One chemical solution for contacting the article to remove the loosely adhering film is comprised of from about 2 to about 10 percent fluoboric acid by volume in water. Solutions below about 2 percent do not remove the loosely adhering film, and solutions above about 10 percent start to attack the more adherent film underlying the loosely adhering film. The solution is at about 25°±5° C and the article is contacted in this solution for about 1 minute ±10 seconds.

Another chemical solution for contacting the article to remove the loosely adhering film is comprised of from about 2 to about 10 percent hydrofluosilicic acid by volume in water. Solutions below about 2 percent do not remove the loosely adhering film, and solutions above about 10 percent start to attack the more adherent film underlying the loosely adhering film. The solution is at about 25°±5° C and the article is contacted in this solution for about 1 minute ±10 seconds.

Removal of the loosely adhering film from the article can also be accomplished by the use of ultrasonic rinsing in water, i.e., submerging the article in water and applying ultrasonic energy in the range of about 20,000 to about 300,000 cycles per second (cps). This is continued for a time of about 1 to 2 minutes or more, or until visual observation shows that no more film is being removed. Below about 20,000 cps, the rate of removal is too slow, and the equipment for running above 300,000 cps involves added expense.

Swabbing the loosely adhering film from the article is done by uniformly rubbing the surface with cotton or paper or other absorbent material, or by brushing the surface with a brush containing natural hog bristles or nylon bristles. In one method cotton swabs or organic swabs such as polyester and nylon swabs are rubbed over the surface of the article. When the article is in the form of a tube the swab is driven through the tube by use of air pressure.

Next, after removal of any loosely adhering film, an optional step of rinsing the article in water can be practiced, preferably using deionized water, to free the article of any residual traces of the material used in removing the loosely adhering film. This step is desirable when one of the chemical solutions has been used.

The article is contacted with an electroless plating solution containing the metal to be deposited on the article upon sufficient contact with the article. Typically the electroless plating solution is flowed uniformly over the surface of the article to enable uniform build up of the metal on the article.

Preferred metals to be deposited on the article of zirconium or a zirconium alloy include copper and nickel, and an especially preferred metal to be deposited on the article is copper.

For depositing copper, an aqueous bath of the following composition has been employed: 3.6 grams/liter of copper sulfate ( $\text{CuSO}_4 \cdot 5\text{H}_2\text{O}$ ), 25 grams/liter sodium potassium tartrate ( $\text{K Na C}_4\text{H}_4\text{O}_6 \cdot 4\text{H}_2\text{O}$ ), 3.8 grams/liter of sodium hydroxide ( $\text{Na OH}$ ), and 10 ml./liter of a 35% formaldehyde solution ( $\text{HCOOH}$ ) with the balance being water. Other proprietary electroless copper plating formulations can be employed such as those identified as MacDermid 9038, Shipley CP 74 and Sel-Rex CU510. The plating bath is agitated and passed uniformly over the article to be plated while being maintained at a temperature of about 50° to about 75° C with a preferred target temperature being 60°±2° C. This procedure produces a very good as-plated adherence with no porosity. In order to insure that the plated article can be used at elevated temperatures without any substantial loss of adhesion, the plated article is out-gassed at a temperature of about 300° to about 400° F (149° to 204° C) for a time period of about 3 hours. In this out-gassing the temperature is raised from ambient to the final temperature at a rate of about 50° F to 125° F per hour.

During the plating of copper on the article, a considerable quantity of hydrogen gas is evolved. The electroless copper plating solution is flowed slowly over the article, and this results in the hydrogen tending to adhere to the wall of the tube. It is necessary to remove this hydrogen gas so that it does not develop back-pressure during plating (i.e., pressure on the surface of the article being plated that stops the plating). The plating process is further facilitated when the surface of the article to be plated is positioned in a vertical position so that evolved hydrogen is swept upward away from the surface being plated.

For plating nickel on zirconium, an aqueous bath of the following composition is employed: 30 grams/liter of nickel chloride ( $\text{Ni Cl}_2 \cdot 6\text{H}_2\text{O}$ ), 10 grams/liter of sodium hypophosphite ( $\text{Na H}_2\text{PO}_2 \cdot \text{H}_2\text{O}$ ), 12.6 grams/liter of sodium citrate ( $\text{Na}_3\text{C}_6\text{H}_5\text{O}_7 \cdot 2\text{H}_2\text{O}$ ), 5 grams/liter of sodium acetate ( $\text{Na C}_2\text{H}_3\text{O}_2$ ) and sufficient sodium hydroxide ( $\text{NaOH}$ ) to give a pH in the range of 4 to 6. Other proprietary electroless nickel plating formulations can be employed such as those identified as En-

plate 410 and Enplate 416. The plating bath is agitated and passed uniformly over the article to be plated while being maintained at a temperature of about 194° to about 212° F (90° to 100° C) with a preferred target temperature being 95°±2° C. This procedure produces a very good as-plated adherence with no porosity. In order to insure that the plated article can be used at elevated temperatures without any substantial loss of adhesion, the same out-gassing procedure employed above for copper is used.

The articles treated by the process of this invention can be zirconium materials taken directly from milling operations or can be articles subjected to prior mechanical cleaning (e.g., grit blasting) or chemically cleaned articles (e.g., cleaned by acid and/or alkaline etching).

Utilizing the foregoing method and the aqueous activating solution, it is possible to obtain a continuous deposit of the metal to be plated on the article of zirconium or a zirconium alloy with a minimum thickness of about 1.5 microns or greater. For best results it is preferred to have a thickness of from about 3 to about 15 microns plated on the article and it is possible to achieve even thicker coatings with the process of this invention. Articles plated by the foregoing process protect the zirconium against most of the usual agents encountered at high temperatures including oxygen, air, water, steam and fission products produced in nuclear fuel elements during nuclear fission.

After the plating it is possible to subject the metal coatings on the article to various treatments including diffusion annealing treatments or plating of a second metal.

The process of this invention produces plated articles having increased adhesion between the plated metal layer and the article. The plated articles of this invention will pass an adhesion test (American Society for Testing Materials Standard B571-72) requiring the test specimen to be bent 180° in repeated cycles until the specimen breaks. Following the fracture of the article, no separation of the deposited metal layer is detected for the articles plated according to the practice of this invention.

The following non-limiting examples illustrate the results obtained in the practice of this invention for achieving coatings upon zirconium articles.

#### EXAMPLE 1

A hollow Zircaloy-2 cladding tube 4 meters in length, 10.7 mm. in inside diameter and 12.4 mm. in outside diameter was plated according to the following procedure. The tube had previously been etched in an acid solution of 50% by weight hydrofluoric acid and 50% by weight nitric acid, contacted with an aqueous 50% by weight sodium hydroxide solution and then rinsed in water.

The tube was cleaned in 1.1.1 trichlorethane, rinsed in deionized water and allowed to dry. The inside surface of the final 7.6±1.3 mm. at each end of the tube was coated with a vinyl lacquer.

Next an aged aqueous activating solution was pumped through the tube at the rate of 1000±200 ml./minute. The solution was comprised of 15 grams/liter of ammonium bifluoride, 0.5 ml./liter sulfuric acid and the balance was deionized water. The solution was aged by immersion of pickled zirconium in the solution for about 10 minutes. This pumping was continued for one minute. The temperature of the solution was

21°±2° C throughout the time the solution was pumped through the tube.

The tube was rinsed by circulating room temperature deionized water through the tube for 1 minute at a flow rate of about 1000±200 ml./minute.

The loosely adhering film (smut) on the inside surface of the tube was removed by immersing the tube in a water bath and applying about 40,000±5000 cycles per second of ultrasonic energy to the tube for 1 minute while deionized water is circulated through the tube. The water leaving the tube is dark and as time passes becomes lighter in color until after 1 minute the water is substantially clean.

The ultrasonic energy was turned off, and the tube was then further rinsed by circulating deionized water (at room temperature) through the tube for 1 minute at a flow rate of about 1000±200 ml./minute.

Next the tube was plated by pumping an electroless copper plating solution through the tube at the rate of 1000±200 ml./minute for 2 hours. The solution was comprised of 3.6 grams/liter of copper sulfate, 25 grams/liter of sodium potassium tartrate, 3.8 grams/liter of sodium hydroxide, 10 ml./liter of formaldehyde and the balance deionized water. The temperature of the plating solution was maintained between 50° and 60° C while being pumped through the tube. The tube was next purged with inert gas (nitrogen) for 1 minute at a flow rate of 3 cubic feet/minute.

The tube was then rinsed by circulating room temperature deionized water through the tube for 5 minutes at a flow rate of about 1000±200 ml./minute.

The tube was air dried and the lacquer was removed from each end with 1.1.1 trichlorethane.

Examination of the tube showed a copper layer of 10 microns in thickness was substantially uniformly plated on the inside surface of the Zircaloy tube, except for the ends masked with the lacquer.

### EXAMPLE 2

The procedure of Example 1 is repeated on another Zircaloy-2 tube of identical dimensions. The process is the same except for a change in the step of removing the loosely adhering film left on the tube after the activation step.

For this example, six cotton swabs were pneumatically forced through the tube at the rate of about 100 meters/second. The first five swabs were observed to be discolored with each succeeding swab showing less discoloration, and the sixth swab being substantially free of any discoloration.

Examination of the tube after the electroless plating step showed a copper layer of 10 microns in thickness was substantially uniformly plated on the inside surface of the Zircaloy tube, except for the ends masked with the lacquer.

### EXAMPLE 3

The procedure of Example 2 is repeated replacing the cotton swabs with six organic swabs prepared by wrapping cylindrical rubber plugs with a single layer of polyester to give a plug diameter of about 10 mm.

The first five swabs were observed to be discolored with each succeeding swab showing less discoloration, and the sixth swab being substantially free of any discoloration.

Examination of the tube after the electroless plating step showed a copper layer of 10 microns in thickness was substantially uniformly plated on the inside surface

of the Zircaloy tube, except for the ends masked with the lacquer.

### EXAMPLE 4

5 The procedure of Example 1 is repeated on another Zircaloy-2 tube of identical dimensions. The process is identical except for a change in the step of removing the loosely adhering film left on the tube after the activation step.

10 For this example an aqueous solution comprised of about 10% fluoboric acid by volume is pumped through the tube at the rate of 1000±200 ml./minute. This was continued for about 1 minute and very effectively removed the loosely adhering film from the tube.

15 Examination of the tube after the electroless plating step showed a copper layer of 10 microns in thickness was substantially uniformly plated in the inside surface of the Zircaloy tube, except for the ends masked with the lacquer.

### EXAMPLE 5

The procedure of Example 1 is repeated on another Zircaloy-2 tube of identical dimensions. The process is identical except for a change in the step of removing the loosely adhering film left on the tube after the activation step.

20 For this Example an aqueous solution comprised of about 10% hydrofluosilicic acid by volume is pumped through the tube at the rate of 1000±200 ml./minute. This was continued for about 1 minute and very effectively removed the loosely adhering film from the tube.

25 Examination of the tube after the electroless plating step showed a copper layer of 10 microns in thickness was substantially uniformly plated on the inside surface of the Zircaloy tube, except for the ends masked with the lacquer.

30 As will be apparent to those skilled in the art, various modifications and changes may be made in the invention described herein. It is accordingly the intention that the invention be construed in the broadest manner within the spirit and scope as set forth in the accompanying claims.

35 What is claimed is:

1. A process for electroless deposition of a metal film on an article comprised of zirconium or a zirconium alloy comprising the steps of

40 (a) activating the article in an aqueous activating solution consisting essentially of from about 10 to about 20 grams per liter of ammonium bifluoride and from about 0.75 to about 2 grams per liter of sulfuric acid, the solution being aged by immersion of pickled zirconium in said solution for about 10 minutes,

45 (b) removing any loosely adhering film formed on the article in the activating step, and

50 (c) contacting the article with an electroless plating solution capable of plating the activated article and containing the metal to be deposited thereon upon sufficient contact with the article.

2. A process according to claim 1 in which the article is rinsed in water after each step of claim 1.

3. A process according to claim 2 in which the water is deionized.

55 4. A process according to claim 1 in which the step of removing the loosely adhering film comprises immersing the article in water and applying ultrasonic energy on the immersed article.

5. A process according to claim 1 in which the step of removing the loosely adhering film comprises contacting the article with an aqueous solution comprising from about 2 to about 10 percent fluoboric acid by volume.

6. A process according to claim 1 in which the step of removing the loosely adhering film comprises contacting the article with an aqueous solution comprising from about 2 to about 10 percent hydrofluosilicic acid by volume.

7. A process according to claim 1 in which the step of removing the loosely adhering film comprises contacting the article with a swab.

8. A process according to claim 7 in which the swab is comprised of an organic material wrapped on a rubber plug.

9. A process according to claim 8 in which the organic material is polyester.

10. A process according to claim 8 in which the organic material is nylon.

11. A process according to claim 7 in which the swab is comprised of cotton.

12. A process according to claim 1 in which the plated article is subsequently out-gassed under a partial vacuum by heating at a temperature in the range of about 300° to about 400° F.

13. A process according to claim 1 in which the article is in the form of a long hollow cylindrical tube comprised of a zirconium alloy.

14. A process for electroless deposition of a metal film on an article comprised of zirconium or a zirconium alloy comprising the steps of

(a) activating the article in an aqueous activating solution consisting essentially of from about 10 to

about 20 grams per liter of ammonium bifluoride and from about 0.75 to about 2 grams per liter of sulfuric acid, the solution being aged by immersion of pickled zirconium in said solution for about 10 minutes,

(b) rinsing the article in water,

(c) removing any loosely adhering film formed on the article in the activating step,

(d) rinsing the article in water, and

(e) contacting the article with an electroless plating solution capable of plating the activated article and containing the metal to be deposited thereon upon sufficient contact with the article.

15. A process according to claim 14 in which the article is in the form of a long hollow cylindrical tube comprised of a zirconium alloy.

16. A process according to claim 14 in which the step of removing the loosely adhering film comprises immersing the article in water and applying ultrasonic energy on the immersed article.

17. A process according to claim 14 in which the step of removing the loosely adhering film comprises contacting the article with an aqueous solution comprising from about 2 to about 10 percent fluoboric acid by volume.

18. A process according to claim 14 in which the step of removing the loosely adhering film comprises contacting the article with an aqueous solution comprising from about 2 to about 10 percent hydrofluosilicic acid by volume.

19. A process according to claim 14 in which the step of removing the loosely adhering film comprises contacting the article with a swab.

\* \* \* \* \*

UNITED STATES PATENT OFFICE  
CERTIFICATE OF CORRECTION

PATENT NO. : 4,093,756  
DATED : 6 June 1978  
INVENTOR(S) : Robert E. Donaghy

It is certified that error appears in the above-identified patent and that said Letters Patent are hereby corrected as shown below:

Column 1, after "Background Of The Invention" insert --The Government has rights in this invention pursuant to Subcontract No. 3-20-46 under Prime Contract EN-77-C-02-4473 awarded by the U.S. Department of Energy.--

Signed and Sealed this

*Sixteenth* Day of *September 1980*

[SEAL]

Attest:

SIDNEY A. DIAMOND

*Attesting Officer*

*Commissioner of Patents and Trademarks*